

[54] **PREVENTION OF HYDROGEN  
EMBRITTLEMENT OF HIGH-STRENGTH  
STEEL BY HYDRAZINE COMPOSITIONS**

[76] Inventors: **James C. Fletcher**, Administrator of the National Aeronautics and Space Administration, with respect to an invention by **Leonard Weber**, Northridge, Calif.

[22] Filed: Sept. 28, 1973

[21] Appl. No.: 401,921

[52] U.S. Cl..... 149/36; 423/407

[51] Int. Cl.<sup>2</sup>..... C06D 5/08

[58] Field of Search..... 149/36; 423/407

[56] **References Cited**

## UNITED STATES PATENTS

2,837,410 6/1958 Haller ..... 423/407

3,421,316 1/1969 Burge et al. ..... 149/36 X

3,710,573 1/1973 Hubbuch et al. ..... 149/36 X

3,740,436 6/1973 Rigsby ..... 423/407  
3,744,971 7/1973 Lamb et al. ..... 149/36 X

**OTHER PUBLICATIONS**

Audrieth et al., "The Chemistry of Hydrazine," pp. 140, 141, 145-148, 213 and 214, John Wiley & Sons, Inc. (1951) New York.

Primary Examiner—Benjamin R. Padgett

Assistant Examiner—E. A. Miller

Attorney, Agent, or Firm—Monte F. Mott; Wilfred Grifka; John R. Manning

[57] **ABSTRACT**

Delayed failure of high-strength steel alloys exposed to compositions containing hydrazine is prevented by addition of potassium hydroxide to the composition in an amount at least sufficient to neutralize acidic impurities. The removal of the acidic impurities eliminates evolution of hydrogen and thus avoids hydrogen embrittlement of the high-strength steel alloys.

7 Claims, No Drawings

**PREVENTION OF HYDROGEN EMBRITTLEMENT  
OF HIGH-STRENGTH STEEL BY HYDRAZINE  
COMPOSITIONS**

**ORIGIN OF THE INVENTION**

The invention described herein was made in the performance of work under a NASA contract and is subject to the provisions of Section 305 of the National Aeronautics and Space Act of 1958, Public Law 83-568 (72 Stat. 435; 42 USC 2457).

**BACKGROUND OF THE INVENTION**

**1. Field of the Invention**

The present invention relates to an improved hydrazine composition and, more particularly, to such a composition capable of long-term contact with high-strength steel surfaces.

**2. Description of the Prior Art**

Steel alloys such as Type 410 Stainless Steel have been found susceptible to delayed failure when exposed to compositions containing acidified hydrazine. Fractography indicates that such failures are similar to known hydrogen embrittlement failures and stress corrosion failures in 410 Stainless Steel. It was found that chemical reactions can occur which release hydrogen at the steel surface. The released hydrogen penetrates the steel and may produce embrittlement or stress corrosion rendering the steel unsuitable for space vehicle tankage and long-term storage.

High-strength steels are highly desirable for space vehicle tankage because of their high-strength/weight ratio, stiffness and ease of manufacture. Such steels, however, are unsuitable for storage tanks for liquid fuel compositions containing hydrazine such as Aerozine-50 in view of the demonstrated incompatibility with acidified hydrazine. The alternative is to fabricate tanks from materials which are not susceptible to hydrogen embrittlement. Aluminum alloys would probably meet these requirements. However, designs to meet required weight limitations would introduce additional complexities and costs. In addition, aluminum tanks are more costly to fabricate because of the greater difficulties encountered in welding, inspection, and repair. An analysis of the embrittlement mechanism indicated that the release of hydrogen on the surface of steel exposed to hydrazine-fuel compositions resulted from reaction between hydrazine, acidic impurities in the hydrazine, and the steel. The acidic impurities, such as CO<sub>2</sub> or Cl<sub>2</sub>, could be present simply from exposure of the fuel to the atmosphere or halogenated solvents. Typical reactions are as follows:

The chemical decomposition of hydrazine results mainly in the formation of nitrogen and ammonia.



Small amounts of hydrogen are also said to be produced in this decomposition but the reaction pathway is obscure. In any event, the amount of hydrogen produced in such autolysis reactions is negligible compared with the large amounts produced in the reaction between steel and the N<sub>2</sub>H<sub>5</sub><sup>+</sup> ion.



This reaction is analogous to the aqueous reaction between hydrogen ion and steel.



The N<sub>2</sub>H<sub>5</sub><sup>+</sup> ion arises from the presence of acidic substances dissolved in the fuel, in the same way that H<sub>3</sub>O<sup>+</sup> is produced from acids dissolved in water:



where HA is a molecule of any acid.

10 In Aerozine-50, the most likely acidic species is carbazic acid, which is formed by reaction of atmospheric carbon dioxide with hydrazine:



Other possible sources of N<sub>2</sub>H<sub>5</sub><sup>+</sup> are ammonium chloride and hydrazinium chloride, both of which may be present in trace amounts.



It should be emphasized that atmospheric carbon dioxide is not the only possible source of acidic impurities in hydrazine-base fuels. For example, halogenated solvents will react with hydrazine to yield hydrazinium salts which act as acids according to the following reaction:



where X is halogen and R is an organic group. Solvents which fall into this category are Freon, trichloroethylene, methylene dichloride and the like.

Thus, it would appear that an obvious solution to 35 counter the hydrogen producing reactions would be the exposure of the hydrazine fuel to basic substances to remove and neutralize the acidic impurities. However, when basic materials such as barium oxide or sodium hydroxide were added to the composition, they were 40 found to form a precipitate which is quite objectionable in respect to contaminating components with small orifices (i.e., valves, injection ports and control systems) unless the treated composition is filtered before storage and prior to use to eliminate the precipitate. Filtering is a very expensive operation and it would be desirable to eliminate it. Furthermore, it would be desirable to have the neutralizing agent present in excess within the composition so that acidic impurities such as carbon dioxide or hydrochloric acid can be continuously neutralized preventing the Aerozine-50 from attacking and degrading the steel (i.e., 410). The excess neutralizing agents such as barium oxide or sodium hydroxide present in the storage tank would react with further amounts of carbon dioxide to form insoluble carbonates which must be filtered and removed before the composition could be sent through the valves or if not properly filtered, the precipitate could clog orifices resulting in catastrophic failures.

60 Austenitic steels and especially weld seams are very susceptible to stress-environment failures when exposed under sustained load to hydrazine liquid fuels.

Experience has shown that fabricated hardware sometimes contain undetected flaws, frequently in welds, and residual stresses resulting from manufacturing operations. In the presence of an aggressive chemical environment, such flaws may grow, causing leaks or catastrophic fracture. Hydrogen permeation testing of

410 Stainless Steel membranes with several surface treatments demonstrated that the treatments failed to completely suppress hydrogen flux generation. The treatments consisted of pickling alone or in combination with distilled water rinses or further in combination with aqueous ammonium fluoride, 8-hydroxy quinoline, perfluoro-octanoic acid, stearic acid or perfluoro-decyl-1-sulfonic acid.

Atomic absorption spectrometry for precipitates suspended in Aerozine-50 following treatment with sieved  $\frac{1}{4}$  inch granular barium oxide revealed approximately 3 ppm barium in the supernatant liquid. Filtration with a 10 micron woven stainless steel wire mesh filter reduced the barium content to 0.9 ppm and further filtration using a 1.0 micron Teflon filter was required to reduce the barium level to 0.6 ppm.

The specifications for the second stage of the Delta rocket entails a first use of a propellant combination of Aerozine-50 and  $N_2O_4$  with Type 410 Stainless Steel tankage. The available published literature does not reveal data establishing compatibility of this fuel combination with 410 Stainless Steel welds. The literature does indicate that 410 parent metal catalyzes decomposition of Aerozine-50 and the two materials when combined in a glass vial. However, sustained load compatibility tests have not been performed with 410 and Aerozine-50. A program was conducted to determine the compatibility of Aerozine-50 and  $N_2O_4$  with 410 Stainless Steel welds under stress, primarily to determine whether Aerozine-50 and/or  $N_2O_4$  would produce flaw extension in welded 410 Stainless Steel stressed in tension.

The program determined that welded specimens of 410 Stainless Steel failed in sustained load within 3 to 30 days exposure to Aerozine-50.  $N_2O_4$  specimens survived the 30-day exposure with no evidence of flaw growth. A number of parameters were investigated to explore their individual and collective effects on time to failure. The parameters included: acidic contaminant condition of the Aerozine-50, test temperature range, method of achieving test temperature range, specimen fuel container material, specimen surface condition, and the number of load cycles supplied to the specimens. An analysis of the data leads to the conclusion that the single most significant factor influencing flaw growth rates and failures is the condition of the fuel.

#### SUMMARY OF THE INVENTION

In accordance with the invention, it has been discovered that addition of potassium hydroxide to hydrazine-containing fuel compositions that are in contact with austenitic steels controls the dissociation constant of hydrazine significantly to reduce and eliminate  $H^+$  ion, i.e., acidity, without forming a precipitate, thus obviating filtration. Both potassium hydroxide and its neutralization reaction products are soluble in hydrazine fuels.

The potassium hydroxide containing hydrazine fuel composition in accordance with the invention prevents corrosion of steel during storage, inhibits decomposition and loss of hydrazine from the stored fuel and permits long-term storage in welded, high-strength, austenitic steel storage tanks under load without fear or danger of acidic impurity induced hydrogen embrittlement or catastrophic fracture.

The acidic impurities may be present in the fuel composition as manufactured or may be absorbed from the

atmosphere during storage or contaminated by halogenated solvents. The potassium hydroxide is added in a minimum concentration necessary to achieve neutrality. For example, Aerozine-50 containing 200 ppm  $CO_2$  requires about 260 to 400 ppm potassium hydroxide for neutralization and stabilization. This is a 1/1 molar ratio and reaction.

The potassium hydroxide may be added in an excess amount over the stoichiometric amount necessary for neutralization in order to accommodate and neutralize further amounts of acidic impurities such as  $CO_2$  which are absorbed from the ambient environment during extended periods of storage. The potassium hydroxide may suitably be added in an amount of 20 to 200 ppm over the amount necessary for neutralization of the as manufactured acidic impurities capable of causing evolution of hydrogen in the presence of austenitic steel surfaces. Typically, potassium hydroxide is added to the fuel in an approximate concentration of 200 ppm to neutralize the acid impurities and/or to maintain the equilibrium in direction of  $N_2H_4$  stability.

The invention is generally applicable to hydrazine-containing compositions such as anhydrous hydrazine, unsymmetrical dimethyl hydrazine (UDMH), mixtures thereof such as Aerozine-50 (A-50), or mixtures with oxidizers such as  $N_2O_4$ . Aerozine-50 has a general composition comprising about 47.76% UDMH, 51.76% hydrazine and 0.36% water. The stress corrosion, hydrogen embrittlement of the composition in presence of austenitic stainless steel was tested by analyzing for diffusion of hydrogen through a steel membrane. The detection technique depends on the observation that hydrogen generated by the reaction of acid at a metal surface diffuses into the metal. This diffusion eventually results in permeation of some hydrogen entirely through the specimen. With a suitable device this hydrogen can be detected as a permeation flux.

The device utilized for testing consisted of two compartments separated by a 0.25 inch steel membrane. This membrane becomes a working electrode of a potentiostat. One of the compartments is filled with 1.0N sodium hydroxide solution. The reference electrode and the auxiliary electrode of the potentiostat are immersed in the sodium hydroxide and the membrane is brought to +100 MVsce. After the membrane has been polarized to equilibrium, the test solution is placed in the other compartment. Hydrogen generated at the membrane surface diffuses through the membrane and is oxidized to  $H^+$  ion by the +100 MVsce. Under the influence of the potential, the  $H^+$  ions migrate to the auxiliary electrode where they are discharged, producing a current flow in the auxiliary circuit. The current is detected as an IR drop across a standard resistor and is displayed on a recorder.

#### EXAMPLE 1

Barium oxide was added to 300 grams of Aerozine-50 until evolution of hydrogen was terminated. The composition was filtered to remove 0.6 ppm of solids.

Carbon dioxide was then generated by combining 0.1 grams of  $Na_2CO_3$  and  $H_2SO_4$ . The evolved  $CO_2$  was trapped and added to 300 grams of Aerozine-50 in an amount of 200 ppm. 51 ml of the  $CO_2$  containing Aerozine-50 composition was treated with 0.1 ml of a 20 g/100 cc KOH solution. The Aerozine-50 was free of carbon dioxide and no hydrogen flux developed. The

composition was clear and no opalescence could be seen.

#### EXAMPLE 2

Example 1 was repeated substituting 0.1 ml of a 20 g/100 cc NaOH solution for the KOH additive. Although the A-50 was free of carbon dioxide and there was no hydrogen flux, an opalescent precipitate developed after 2 minutes.

It is to be understood that only preferred embodiments of the invention have been described and that numerous substitutions, alterations and modifications are all permissible without departing from the spirit and scope of the invention as defined in the following claims.

What is claimed is:

1. A stabilized composition compatible with high-strength steel surfaces consisting essentially of a hydrazine containing material selected from the group consisting of substantially anhydrous hydrazine, unsymmetrical dimethyl hydrazine, and mixtures thereof, said material containing acidic impurities, and a minor amount of potassium hydroxide at least sufficient to neutralize said impurities.

2. A composition according to claim 1 in which potassium hydroxide is present in an amount of 260 to 400 ppm for 200 ppm of CO<sub>2</sub> impurity.

3. A composition according to claim 1 in which the potassium hydroxide is present in an amount of 20 to 200 ppm over the amount necessary to stoichiometrically neutralize the impurities present in the composition at the time of addition of the potassium hydroxide.

4. A method of stabilizing an acid impurity contaminated hydrazine containing composition from evolution of hydrogen without the formation of a precipitate, said hydrazine containing composition selected from the group consisting of substantially anhydrous hydrazine, unsymmetrical dimethyl hydrazine, and mixtures thereof, comprising;

15 adding potassium hydroxide to said composition in a minor amount at least sufficient to neutralize said impurities.

5. A method according to claim 4 further comprising the step of placing said stabilized composition in contact with the surface of austenitic steel.

6. A method according to claim 5 in which the potassium hydroxide is added in an amount of 260 to 400 ppm for 200 ppm of CO<sub>2</sub> impurity.

7. A method according to claim 5 in which the potassium hydroxide is added in an amount of 20 to 200 ppm over the amount necessary to stoichiometrically neutralize the impurities present in the composition at the time of addition of the potassium hydroxide.

\* \* \* \* \*

30

35

40

45

50

55

60

65